# EUROPEAN PATENT SPECIFICATION

(11) **EP 2 685 475 B1**
(45) Date of publication and mention of the grant of the patent: **21.08.2019**
(21) Application number: 12803474.1
(22) Date of filing: 15.03.2012
(51) Int. Cl.: H01F 1/08, B22F 3/22, C22C 33/02, C22C 38/00, H01F 1/057, H01F 41/02

(54) **METHOD FOR MANUFACTURING RARE EARTH PERMANENT MAGNET**
VERFAHREN ZUR HERSTELLUNG EINES SELTENERD-PERMANENTMAGNETEN
PROCÉDÉ DE FABRICATION D'UN AIMANT PERMANENT AUX TERRES RARES

(30) Priority: 24.06.2011 JP 2011140911
(43) Date of publication of application: 15.01.2014
(73) Proprietor: Nitto Denko Corporation, Ibaraki-shi, Osaka 567-8680 (JP)
(72) Inventor: OZEKI, Izumi, Ibaraki-shi Osaka 567-8680 (JP); KUME, Katsuya, Ibaraki-shi Osaka 567-8680 (JP); OKUNO, Toshiaki, Ibaraki-shi Osaka 567-8680 (JP); OZAKI, Takashi, Ibaraki-shi Osaka 567-8680 (JP); OMURE, Tomohiro, Ibaraki-shi Osaka 567-8680 (JP); TAIHAKU, Keisuke, Ibaraki-shi Osaka 567-8680 (JP)
(74) Representative: Grünecker Patent- und Rechtsanwälte PartG mbB
(86) International application number: PCT/JP2012/056713
(87) International publication number: WO 2012/176513

(56) References cited:
- JP-A- H10 163 055
- JP-A- 2005 197 299
- JP-A- 2005 197 299
- JP-A- 2005 203 555
- JP-A- 2007 134 417
- JP-A- 2007 296 502
- JP-A- 2009 259 955
- JP-A- 2009 267 221
- US-A1- 2003 062 097

## Description

### TECHNICAL FIELD

The present invention relates to a manufacturing method of the rare-earth permanent magnet.

### BACKGROUND ART

In recent years, a decrease in size and weight, an increase in power output and an increase in efficiency have been required in a permanent magnet motor used in a hybrid car, a hard disk drive. To realize such a decrease in size and weight, an increase in power output and an increase in efficiency in the permanent magnet motor mentioned above, film-thinning and a further improvement in magnetic performance have been required of a permanent magnet to be buried in the permanent magnet motor.

Here, as a method for manufacturing the permanent magnet used in the permanent magnet motor, a powder sintering method is generally used. In the powder sintering method as used herein, a raw material is first pulverized with a jet mill (dry-milling) to produce a magnet powder. Thereafter, the magnet powder is placed in a mold, and press molded to a desired shape while a magnetic field is applied from the outside. Then, the solid magnet powder molded into the desired shape is sintered at a predetermined temperature (for example, 1100 degrees Celsius in a case of an Nd-Fe-B-based magnet), thereby manufacturing the permanent magnet.

However, when the permanent magnet is manufactured by the above-mentioned powder sintering method, there have been the following problems. That is to say, in the powder sintering method, it is necessary to secure a predetermined porosity in a press-molded magnet powder in order to perform magnetic field orientation. However, if the magnet powder having the predetermined porosity is sintered, it is difficult to uniformly contract at the time of sintering. Accordingly deformations such as warpage and depressions occur after sintering. Further, since pressure unevenness occurs at the time of pressing the magnet powder, the magnet is formed to have inhomogeneous density after sintering to generate distortion on a surface of the magnet. Conventionally, it has therefore been required to compression-mold the magnet powder to a larger size than that of a desired shape, assuming that the surface of the magnet has some distortion. Then, diamond cutting and polishing operations have been performed after sintering, for alteration to the desired shape. As a result, the number of manufacturing processes increases, and there also is a possibility of deteriorating qualities of the permanent magnet manufactured.

Specifically, when a thin-film magnet is cut out of a bulk body having a larger size as discussed above, material yield is significantly decreased. Further, a problem of large increase in man-hours has also been raised.

Therefore, as a means for solving the above problems, there has been proposed a method of manufacturing a permanent magnet through kneading a magnet powder and a binder, preparing a green sheet, and sintering the green sheet thus prepared (for instance, Japanese Laid-open Patent Application Publication No. 1-150303) .

### PRIOR ART DOCUMENT

### PATENT DOCUMENT

Patent document 1: Japanese Laid-open Patent Application Publication No. 1-150303 (pages 3 and 4)

JP 2009 267221 A describes a manufacturing method for a magnet comprising a magnetic powder containing a three component-type neodynium with added iron and boron having a high degree of particle orientation and uniform density at high manufacturing yield.

JP H10 163055 A describes a method for a permanent magnet having raised magnetic characteristics and electric resistance in which a specified magnet powder is mixed with a binder and insulator, a powder is formed, following a de-binding and compacting step.

JP 2005 197299 A discloses a manufacturing method of a permanent magnet containing a rare earth element, a transition metal element and boron in which a forming body is subjected to debindering treatment by resistance heating before sintering by discharge plasma sintering.

US 2003/062097 A1 describes a Nd-Fe-B type rare earth magnet alloy with hard magnetic phases and soft magnetic phases. The magnet alloy is obtained using a strip casting method or ultra cooling method and serves as material for an anisotropic exchange spring magnet to be applied to a motor.

### DISCLOSURE OF THE INVENTION

### PROBLEM TO BE SOLVED BY THE INVENTION

Here, in a case of forming the magnet powder into a green sheet as in the above Patent Document 1, it is industrially important to improve thickness precision of the green sheet. One of the reasons for this is that, when a plurality of magnets are sintered simultaneously in order to boost productivity, low precision in the green sheet thickness leads to variations in temperatures to properly sinter individual magnets, resulting in unsatisfactory sintering of the plurality of magnets as total homogeneous quality. Especially in a case of performing pressure sintering as the sintering method, the low precision of the thickness should also lead to variations of proper values to press the green sheet. However, it has been difficult to achieve high precision in green sheet thickness with conventional methods for manufacturing a green sheet such as injection molding, metal molding or a doctor blade system.

Meanwhile, it has been known that the magnetic performance of a permanent magnet can be basically improved by making the crystal grain size in a sintered body very fine, because the magnetic characteristic of a magnet can be approximated by a theory of a single-domain particles. Here, in order to make the grain size in the sintered body very fine, a particle size of the magnet raw material before sintering also needs to be made very fine. However, even if the magnet raw material finely milled into a very fine particle size is compacted and sintered, grain growth occurs in the magnet particles at the time of sintering. Therefore, after sintering, the crystal grain size in the sintered body increases to be larger than the size before sintering, and as a result, it has been impossible to achieve a very fine crystal grain size. In addition, if the crystal grain has a larger size, the domain walls created in the grain easily move and reverse magnetic domain increases in volume, resulting in drastic decrease of the coercive force.

The present invention has been made in order to solve the above-mentioned conventional problems, and an object the invention is to provide a manufacturing method of the rare-earth permanent magnet capable of achieving inhibition of grain growth at sintering by forming the magnet powder into a green sheet and sintering the thus formed green sheet by pressure sintering as well as improvement of thickness precision of the green sheet by high-precision coating of the mixture of the magnet powder and the binder over a substrate, so that productivity can be improved.

### MEANS FOR SOLVING THE PROBLEM

This object is solved with the manufacturing method of claim 1. Preferred embodiments are defined in the subclaims 2 to 5 as well as in the description.

To achieve the above object, the present invention provides a manufacturing method of a rare-earth permanent magnet comprising the steps of: milling magnet material into magnet powder; preparing a mixture by mixing the magnet powder and a binder so that the binder is included at a rate of 1 to 40 wt% with reference to total weight of the magnet powder and the binder; obtaining a green sheet by coating a surface of a substrate with the mixture by high precision coating so that a sheet-like-shaped green sheet has thickness precision within a margin of error of plus or minus 5% with reference to a designed value; and pressure sintering the green sheet.

In the above-described manufacturing method of a rare-earth permanent magnet of the present invention, in the step of obtaining the green sheet, the substrate is coated with the mixture by using a slot die, and thickness of the green sheet thus coated with the mixture is measured so as to perform feed back control of a gap between the slot die and the substrate based on a measured thickness.

In the above-described manufacturing method of a rare-earth permanent magnet of the present invention, in the step of pressure sintering the green sheet, the green sheet is sintered by uniaxial pressure sintering.

In the above-described manufacturing method of a rare-earth permanent magnet of the present invention, in the step of pressure sintering the green sheet, the green sheet is sintered by electric current sintering.

In the above-described manufacturing method of a rare-earth permanent magnet of the present invention, before the step of pressure sintering the green sheet, the binder is decomposed and removed from the green sheet by holding the green sheet for a predetermined length of time at binder decomposition temperature in a non-oxidizing atmosphere.

In the above-described manufacturing method of a rare-earth permanent magnet of the present invention, when decomposing and removing the binder from the green sheet, the green sheet is held for the predetermined length of time at temperature range of 200 degrees Celsius to 900 degrees Celsius in a hydrogen atmosphere or a mixed gas atmosphere of hydrogen and inert gas.

### EFFECT OF THE INVENTION

According to the manufacturing method of a rare-earth permanent magnet of the present invention, magnet powder and a binder are mixed to obtain a mixture including 1 to 40 wt% of the binder therein and a green sheet is obtained by high precision coating of a substrate with the mixture so that a sheet-like-shaped green sheet has thickness precision within a margin of error of plus or minus 5% with reference to a designed value. Accordingly, even if a plurality of formed bodies die-cut from the green sheet are sintered simultaneously, the formed bodies can be sintered satisfactorily; the thickness of each formed body is made uniform, which avoids variations in proper pressure values or proper sintering temperatures. As a result, improvement in productivity can be achieved. Further, the rare-earth permanent magnet is a pressure-sintered magnet made of the green sheet. Therefore, the thus sintered green sheet can suppress grain growth at sintering to improve magnetic performance. Further, the thus obtained permanent magnet uniformly contracts and deformations such as warpage and depressions do not occur there. Further, the sintered green sheet having uniformly contracted gets pressed uniformly, which eliminates adjustment process to be conventionally performed after sintering and simplifies manufacturing process. Thereby, a permanent magnet can be manufactured with dimensional accuracy. Further, even if above such permanent magnets are made thin in the course of manufacturing, increase in the number of manufacturing processes can be avoided without lowering a material yield.

Further, according to the manufacturing method of a rare-earth permanent magnet of the present invention, in the step of obtaining the green sheet, thickness of the green sheet thus coated with the mixture is measured so as to perform feed back control of a gap between the slot die and the substrate based on a measured thickness. Therefore, the thickness precision of the green sheet can further be improved.

Further, according to the manufacturing method of a rare-earth permanent magnet of the present invention, in the step of pressure sintering the green sheet, the green sheet is sintered by uniaxial pressure sintering. Therefore, the thus sintered green sheet uniformly contracts and deformations such as warpage and depressions can be prevented in the sintered green sheet.

Further, according to the manufacturing method of a rare-earth permanent magnet of the present invention, in the step of pressure sintering the green sheet, the green sheet is sintered by electric current sintering. Thereby, quick heating and cooling can be realized and sintering in a lower temperature range can be realized, as well. As a result, the heating-up and holding periods in the sintering process can be shortened; so that a densely sintered body can be manufactured in which grain growth of the magnet particle is suppressed.

Further, according to the manufacturing method of a rare-earth permanent magnet of the present invention, before the step of pressure sintering the green sheet, the binder is decomposed and removed from the green sheet by holding the green sheet for a predetermined length of time at binder decomposition temperature in a non-oxidizing atmosphere. Thereby, carbon content in the magnet can be reduced previously. Consequently, previous reduction of carbon content can prevent alpha iron from separating out in a main phase of the sintered magnet and the entirety of the magnet can be sintered densely. Thereby, decrease in the coercive force can be prevented.

Further, according to the manufacturing method of a rare-earth permanent magnet of the present invention, the green sheet to which the binder has been mixed is held in a hydrogen atmosphere or a mixed gas atmosphere of hydrogen and inert gas. Thereby, carbon content in the magnet can be reduced reliably.

### BRIEF DESCRIPTION OF THE DRAWINGS

[Fig. 1] is an overall view of a permanent magnet according to the invention.
[Fig. 2] is a view depicting an effect at sintering on a basis of improved thickness precision in a green sheet according to the invention.
[Fig. 3] is a view depicting a problem at sintering with lower thickness precision in the green sheet according to the invention.
[Fig. 4] is an explanatory diagram illustrating manufacturing processes of a permanent magnet according to the invention.
[Fig. 5] is an explanatory diagram specifically illustrating a formation process of the green sheet in the manufacturing process of the permanent magnet according to the invention.
[Fig. 6] is an explanatory diagram specifically illustrating a pressure sintering process of the green sheet in the manufacturing process of the permanent magnet according to the invention.

### BEST MODE FOR CARRYING OUT THE INVENTION

A specific embodiment of a method for manufacturing the rare-earth permanent magnet according to the present invention will be described below in detail with reference to the drawings.

### [Constitution of Permanent Magnet]

First, a constitution of a permanent magnet 1 according to the present invention will be described. Fig. 1 is an overall view of the permanent magnet 1 according to the present invention. Incidentally, the permanent magnet 1 depicted in Fig. 1 has a fan-like shape; however, the shape of the permanent magnet 1 may be changed according to the shape of a cutting-die.

As the permanent magnet 1 according to the present invention, an Nd-Fe-B-based magnet may be used. Incidentally, the contents of respective components are regarded as Nd: 27 to 40 wt%, B: 1 to 2 wt%, and Fe (electrolytic iron) : 60 to 70 wt%. Furthermore, the permanent magnet 1 may include other elements such as Dy, Tb, Co, Cu, Al, Si, Ga, Nb, V, Pr, Mo, Zr, Ta, Ti, W, Ag, Bi, Zn or Mg in small amount, in order to improve the magnetic properties thereof. Fig. 1 is an overall view of the permanent magnet 1 according to the present embodiment.

The permanent magnet 1 as used herein is a thin film-like permanent magnet having a thickness of 0.05 to 10 mm (for instance, 4 mm), and is prepared by pressure sintering a formed body (a green sheet) formed into a sheet-like shape from a mixture (a slurry or a powdery mixture) of magnet powder and a binder as described later.

Meanwhile, as the means for pressure sintering the green sheet, there are hot pressing, hot isostatic pressing (HIP), high pressure synthesis, gas pressure sintering, spark plasma sintering (SPS), for instance. However, it is desirable to adopt a method where sintering is performed in a shorter duration and at a lower temperature, so as to prevent grain growth of the magnet particles during the sintering. It is also desirable to adopt a sintering method capable of suppressing warpage formed in the sintered magnets. Accordingly, specifically in the present invention, it is preferable to adopt the SPS method which is uniaxial pressure sintering in which pressure is uniaxially applied and also in which sintering is performed by electric current sintering, from among the above sintering methods.

Here, the SPS method is a method of heating a graphite sintering die with a sintering object arranged inside while pressurizing in a uniaxial direction. The SPS method utilizes pulse heating and mechanical pressure application, so that the sintering is driven complexly by electromagnetic energy by pulse conduction, self-heating of the object to be processed and spark plasma energy generated among particles, in addition to thermal or mechanical energy used for ordinary sintering. Accordingly, quicker heating and cooling can be realized, compared with atmospheric heating by an electric furnace, and sintering at a lower temperature range can also be realized. As a result, the heating-up and holding periods in the sintering process can be shortened, making it possible to manufacture a densely sintered body in which grain growth of the magnet particles is suppressed. Further, the sintering object is sintered while being pressurized in a uniaxial direction, so that the warpage after sintering can be suppressed.

Furthermore, the green sheet is die-cut into a desired product shape (for instance, a fan-like shape shown in Fig. 1) to obtain a formed body and the formed body is arranged inside the sintering die of the SPS apparatus, upon executing the SPS method. According to the present invention, a plurality of formed bodies (for instance, ten formed bodies) 2 are arranged inside the sintering die 3 at a time, as depicted in Fig. 2, in order to boost the productivity. Here, in the present invention, the green sheet is configured to have thickness precision within a margin of error of plus or minus 5 %, preferably plus or minus 3 %, or more preferably plus or minus 1 %, with reference to a designed value. As a result, according to the present invention, as the thickness d of each formed body 2 is uniform, there are no variations in proper pressure values or proper heating temperatures of respective formed bodies 2 and the sintering can be performed satisfactorily even in a case where a plurality of formed bodies (for instance, ten formed bodies) 2 are arranged inside the sintering die 3 and sintered at a time, as illustrated in Fig. 2. Meanwhile, if the green sheet is formed with low precision in thickness (for instance, more than plus or minus 5 % with reference to the designed value), the thickness d of each formed body 2 is not uniform in the case where a plurality of formed bodies (for instance, ten formed bodies) 2 are arranged inside the sintering die 3 and sintered at a time as illustrated in Fig. 3. Accordingly, imbalanced pulse current passes through the respective formed bodies 2 and there occur variations in proper pressure values or proper heating temperatures and the sintering cannot be performed satisfactorily. Incidentally, in the case where the plurality of formed bodies 2 are simultaneously sintered, there may be employed an SPS apparatus having a plurality of sintering dies. There, formed bodies 2 may be respectively placed in the plurality of sintering dies of the SPS apparatus and then simultaneously sintered.

In the present invention, when preparing a green sheet, resin, long-chain hydrocarbon, fatty acid methyl ester or a mixture thereof is used as the binder to be mixed with the magnet powder.

Further, if the resin is used as the binder, there are preferably used, for instance, polyisobutylene (PIB), butyl rubber (IIR), polyisoprene (IR), polybutadiene, polystyrene, styrene-isoprene block copolymer (SIS), styrene-butadiene block copolymer (SBS), Poly(2-methyl-1-pentene), poly(2-methyl-1-butene), poly(alpha-methylstyrene), polybutylmethacrylate, polymethylmethacrylate. Incidentally, low molecular weight polyisobutylene is preferably added to the poly(alpha-methylstyrene) to produce flexibility. Further, as resin used for the binder, there are preferably used a polymer containing no oxygen and exhibiting depolymerization property (for instance, polyisobutylene) to reduce the oxygen content contained in the magnet.

Incidentally, in a case slurry-molding is employed for forming the green sheet, the binder is preferably made of a resin excluding polyethylene and polypropylene so that the binder can get dissolved in a general purpose solvent such as toluene or like. Meanwhile, in a case hot-melt molding is employed for forming the green sheet, a thermoplastic resin is preferably used for the convenience of performing magnetic field orientation using the formed green sheet in a heated and softened state.

Meanwhile, in a case a long-chain hydrocarbon is used for the binder, there is preferably used a long-chain saturated hydrocarbon (long-chain alkane) being solid at room temperature and being liquid at a temperature higher than the room temperature. Specifically, a long-chain saturated hydrocarbon whose carbon number is 18 or more is preferably used. In the case of using the hot melt molding when forming the green sheet, the magnetic field orientation of the green sheet is performed in a state where the green sheet is heated to soften at a temperature higher than the melting point of the long-chain hydrocarbon.

In a case where a fatty acid methyl ester is used for the binder, there are preferably used methyl stearate, methyl docosanoate, being solid at room temperature and being liquid at a temperature higher than the room temperature in a similar manner to the case using long-chain hydrocarbon. In the case of using the hot melt molding when forming the green sheet, the magnetic field orientation of the green sheet is performed in a state where the green sheet is heated to soften at a temperature higher than the melting point of fatty acid methyl ester.

Further, the amount of the binder to be added is an appropriate amount to fill the gaps between magnet particles so that thickness precision of the sheet can be improved when forming the mixture of the magnet powder and the binder into a sheet-like shape. For instance, the binder proportion to the amount of magnet powder and binder in total in the slurry after the addition of the binder is preferably 1 to 40 wt%, more preferably 2 to 30 wt%, still more preferably 3 to 20 wt%.

### [Method for Manufacturing Permanent Magnet]

Next, a method for manufacturing the permanent magnet 1 according to the present invention will be described below with reference to Fig. 4. Fig. 4 is an explanatory view illustrating a manufacturing process of the permanent magnet 1 according to the present invention.

First, there is manufactured an ingot comprising Nd-Fe-B of certain fractions (for instance, Nd: 32.7 wt%, Fe (electrolytic iron) : 65.96 wt%, and B: 1.34 wt%). Thereafter the ingot is coarsely milled using a stamp mill, a crusher to a size of approximately 200 µm. Otherwise, the ingot is dissolved, formed into flakes using a strip-casting method, and then coarsely milled using a hydrogen pulverization method.

Next, the coarsely milled magnet powder is finely milled with a jet mill 11 to form fine powder of which the average particle diameter is smaller than a predetermined size (for instance, 1.0 µm through 5.0 µm) in: (a) an atmosphere composed of inert gas such as nitrogen gas, argon (Ar) gas, helium (He) gas having an oxygen content of substantially 0 %; or (b) an atmosphere composed of inert gas such as nitrogen gas, Ar gas, He gas having an oxygen content of 0.0001 through 0.5 %. Here, the term "having an oxygen content of substantially 0 %" is not limited to a case where the oxygen content is completely 0 %, but may include a case where oxygen is contained in such an amount as to allow a slight formation of an oxide film on the surface of the fine powder. Incidentally, wet-milling may be employed for a method for milling the magnet material. For instance, in a wet method using a bead mill, using toluene as a solvent, coarsely milled magnet powder may be finely milled to a predetermined size (for instance, 0.1 µm through 5.0 µm). Thereafter, the magnet powder contained in the organic solvent after the wet milling may be desiccated by such a method as vacuum desiccation to obtain the desiccated magnet powder. There may be configured to add and knead the binder to the organic solvent after the wet milling without removing the magnet powder from the organic solvent to obtain later described slurry 12.

Through using the above wet-milling, the magnetic material can be milled into still smaller grain sizes than those in the dry-milling. However, if the wet-milling is employed, there rises a problem of residual organic compounds in the magnet due to the organic solvent, even if the later vacuum desiccation vaporizes the organic solvent. However, this problem can be solved by removing carbons from the magnet through performing the later-described calcination process to decompose the organic compounds remaining with the binder by heat.

Meanwhile, a binder solution is prepared for adding to the fine powder finely milled by the jet mill 11. Here, as mentioned above, there can be used a resin, a long-chain hydrocarbon, fatty acid methyl ester or a mixture thereof as binder. Then, binder solution is prepared through dissolving the binder into a solvent. The solvent to be used for dissolving is not specifically limited, and may include: alcohols such as isopropyl alcohol, ethanol and methanol; lower hydrocarbons such as pentane and hexane; aromatic series such as benzene, toluene and xylene; esters such as ethyl acetate; ketones; and a mixture thereof. However, toluene or ethyl acetate is used here.

Successively, the above binder solution is added to the fine powder classified at the jet mill 11. Through this, slurry 12 in which the fine powder of magnet raw material, the binder and the organic solvent are mixed is prepared. Here, the amount of binder solution to be added is preferably such that binder proportion to the amount of magnet powder and binder in total in the slurry after the addition is 1 to 40 wt%, more preferably 2 to 30 wt%,still more preferably 3 to 20 wt%. For instance, 100 grams of 20 wt% binder solution is added to 100 grams of the magnet powder to prepare the slurry 12. Here, the addition of the binder solution is performed in an atmosphere composed of inert gas such as nitrogen gas, Ar gas or He gas.

Subsequently, a green sheet 13 is formed from the slurry 12 thus produced. The green sheet 13 may be formed by, for instance, a coating method in which the produced slurry 12 is spread on a supporting substrate 14 such as a separator as needed by an appropriate system and then desiccated. Incidentally, the coating method is preferably a method excellent in layer thickness controllability, such as a doctor blade system, a slot-die system, or a comma coating system. For realizing thickness precision, a slot-die system or a comma coating system is especially favorable as being excellent in layer thickness controllability (as being a method capable of applying a layer with accurate thickness on a surface of a substrate). For instance, the following embodiment adopts a slot-die system. As supporting substrate 14, a silicone-treated polyester film is used. Further, a green sheet 13 is dried by holding it at 90 degrees Celsius for 10 minutes and subsequently at 130 degrees Celsius for 30 minutes. Further, a defoaming agent may preferably be used in conjunction therewith to sufficiently perform defoaming treatment so that no air bubbles remain in a spread layer.

Here will be given a detailed description of the formation process of a green sheet 13 using a slot-die system referring to Fig. 5. Fig. 5 is an explanatory diagram illustrating the formation process of the green sheet 13 using the slot-die system.

As illustrated in Fig. 5, a slot die 15 used for the slot-die system is formed by putting blocks 16 and 17 together. There, a gap between the blocks 16 and 17 serves as a slit 18 and a cavity (liquid pool) 19. The cavity 19 communicates with a die inlet 20 formed in the block 17. Further, the die inlet 20 is connected with a slurry feed system configured with a metering pump (not shown), and the cavity 19 receives the feed of metered slurry 12 through the die inlet 20 by the metering pump. Further, the slurry 12 fed to the cavity 19 is delivered to the slit 18, and discharged at a predetermined coating width from a discharge outlet 21 of the slit 18, with a pressure which is uniform in transverse direction in a constant amount per unit of time. Meanwhile, a supporting substrate 14 is conveyed along the rotation of a coating roll 22 at a predetermined speed. As a result, the discharged slurry 12 is laid down on the supporting substrate 14 with a predetermined thickness.

Further, in the formation process of the green sheet 13 by the slot-die system, it is desirable to measure the actual sheet thickness of the green sheet 13 after coating, and to perform feed back control of a gap D between the slot die 15 and the supporting substrate 14 based on the measured thickness. Further, it is desirable to minimize the variation in feed rate of the slurry supplied to the slot die 15 (for instance, suppress the variation within plus or minus 0.1 %), and in addition, to also minimize the variation in coating speed (for instance, suppress the variation within plus or minus 0.1 %) . As a result, thickness precision of the green sheet can further be improved. Incidentally, the thickness precision of the formed green sheet is within a margin of error of plus or minus 5 % with reference to a designed value (for instance, 4 mm), preferably within plus or minus 3 %, or more preferably within plus or minus 1 %.

Incidentally, a preset thickness of the green sheet 13 is desirably within a range of 0.05 mm through 10 mm. If the thickness is set to be thinner than 0.05 mm, it becomes necessary to accumulate many layers, which lowers the productivity. Meanwhile, if the thickness is set to be thicker than 10 mm, it becomes necessary to decrease the drying rate so as to inhibit air bubbles from forming at drying, which significantly lowers the productivity.

Further, when mixing the magnet powder with the binder, the mixture may be made into not the slurry 12, but a mixture in the form of powder (hereinafter referred to as a powdery mixture) made of the magnet powder and the binder without adding the organic solvent. There may be employed hot melt coating in which the powdery mixture is heated to melt, and turns into a fluid state and then is spread onto the supporting substrate 14 such as the separator. The mixture spread by the hot melt coating is left to cool and solidify, so that the green sheet 13 can be formed in a long sheet fashion on the supporting substrate 14. Incidentally, the temperature for heating and melting the powdery mixture differs depending on the kind or amount of binder to be used, but is set here at 50 through 300 degrees Celsius. However, it is necessary to set the temperature higher than the melting point of the binder to be used. Here, in order to mix the magnet powder and the binder together, the magnet powder and the binder are, for instance, separately put into an organic solvent and stirred with a stirrer. After stirring, the organic solvent containing the magnet powder and the binder is heated to vaporize the organic solvent, so that the powdery mixture is extracted. Further, specifically when the magnet powder is milled by a wet method, there may be employed a configuration in which, without isolating the magnet powder out of an organic solvent used for the milling, the binder is added to the organic solvent and kneaded, and thereafter the organic solvent is vaporized to obtain the powdery mixture.

Further, a pulsed field is applied before drying to the green sheet 13 coated on the supporting substrate 14, in a direction intersecting a transfer direction. The intensity of the applied magnetic field is 397.89 [kAm⁻¹] (5000[Oe]) through 11936.62 [kAm⁻¹] (150000[Oe]), or preferably 795.77 [kAm⁻¹] (10000[Oe]) through 9549.30 [kAm⁻¹] (120000[Oe]). Incidentally, the direction to orient the magnetic field needs to be determined taking into consideration the magnetic field direction required for the permanent magnet 1 formed from the green sheet 13, but is preferably in-plane direction. Incidentally, if the green sheet is formed by the hot melt molding, the magnetic field orientation of the green sheet is performed in a state where the green sheet is heated to soften in a temperature above the glass transition point or the melting point of the binder. Further, the magnetic field orientation may be performed before the formed green sheet has congealed.

Then, the green sheet 13 made from the slurry 12 is die-cut into a desired product shape (for example, the fan-like shape shown in Fig. 1) to form a formed body 25.

Thereafter, the formed body 25 thus formed is held at a binder-decomposition temperature for several hours (for instance, five hours) in a non-oxidizing atmosphere (specifically in this invention, a hydrogen atmosphere or a mixed gas atmosphere of hydrogen and inert gas) and a calcination process in hydrogen is performed. The hydrogen feed rate during the calcination is, for instance, 5 L/min, if the calcination is performed in the hydrogen atmosphere. By the calcination process in hydrogen, the binder can be decomposed into monomers through depolymerization reaction, released therefrom and removed. Namely, so-called decarbonization is performed in which carbon content in the formed body 25 is reduced. Furthermore, calcination process in hydrogen is to be performed under such a condition that carbon content in the formed body 25 is 1500 ppm or lower, or more preferably 1000 ppm or lower. Accordingly, it becomes possible to densely sinter the permanent magnet 1 as a whole in the following sintering process, and the decrease in the residual magnetic flux density or in the coercive force can be prevented.

The binder-decomposition temperature is determined based on the analysis of the binder decomposition products and decomposition residues. In particular, the temperature range to be selected is such that, when the binder decomposition products are trapped, no decomposition products except monomers are detected, and when the residues are analyzed, no products due to the side reaction of remnant binder components are detected. The temperature differs depending on the type of binder, but may be set at 200 through 900 degrees Celsius, or more preferably 400 through 600 degrees Celsius (for instance, 600 degrees Celsius).

Further, in a case the magnet raw material is milled in an organic solvent by wet-milling, the calcination process is performed at a decomposition temperature of the organic compound composing the organic solvent as well as the binder decomposition temperature. Accordingly, it is also made possible to remove the residual organic solvent. The decomposition temperature for an organic compound is determined based on the type of organic solvent to be used, but basically the organic compound can be thermally decomposed in the above binder decomposition temperature.

Thereafter, a sintering process is performed in which the formed body 25 calcined in the calcination process in hydrogen is sintered. In the present invention, pressure sintering is applied to the calcined formed body 25. The pressure sintering includes, for instance, hot pressing, hot isostatic pressing (HIP), high pressure synthesis, gas pressure sintering, spark plasma sintering (SPS). However, it is preferable to adopt the spark plasma sintering which is uniaxial pressure sintering in which pressure is uniaxially applied and also in which sintering is preformed by electric current sintering so as to prevent grain growth of the magnet particles during the sintering and also to prevent warpage formed in the sintered magnets.

Here will be given a detailed description of the pressure sintering process of a formed body 25 using the SPS method, referring to Fig. 6. Fig. 6 is a schematic diagram depicting the pressure sintering process of the formed body 25 using the SPS method.

When performing the spark plasma sintering as illustrated in Fig. 6, first, the formed body 25 is put in a graphite sintering die 31. Incidentally, the above calcination process in hydrogen may also be performed under the state where the formed body 25 is put in the sintering die 31. Then, the formed body 25 put in the sintering die 31 is held in a vacuum chamber 32, and an upper punch 33 and a lower punch 34 also made of graphite are set thereat. After that, using an upper punch electrode 35 coupled to the upper punch 33 and a lower punch electrode 36 coupled to the lower punch 34, pulsed DC voltage/current being low voltage and high current is applied. At the same time, a load is applied to the upper punch 33 and the lower punch 34 from upper and lower directions using a pressurizing mechanism (not shown). As a result, the formed body 25 put inside the sintering die 31 is sintered while being pressurized. Further, the spark plasma sintering is preferably executed to a plurality of formed bodies (for instance, ten formed bodies) 25 simultaneously, so that the productivity may be improved. Incidentally, at the simultaneous spark plasma sintering to the plurality of formed bodies 25, the plurality of formed bodies 25 may be put in one sintering die 31, or may be arranged in different sintering dies 31, respectively. Incidentally, in the case that the plurality of formed bodies 25 are respectively arranged in different sintering dies 31, an SPS apparatus provided with a plurality of sintering dies 31 is used to execute sintering. There, the upper punch 33 and the lower punch 34 for pressing the formed bodies 25 are configured to be integrally used for the plurality of sintering dies 31 (so that the pressure can be applied simultaneously by the upper punch 33 and the lower punch 34) which are integrally-moving).

Incidentally, the detailed sintering condition is as follows:
Pressure value: 30 MPa
Sintering temperature: raised by 10 deg. C. per min. up to 940 deg. C. and held for 5 min.
Atmosphere: vacuum atmosphere of several Pa or lower.

After the spark plasma sintering, the formed body 25 is cooled down, and again undergoes a heat treatment in 600 through 1000 degrees Celsius for two hours. As a result of the sintering, the permanent magnet 1 is manufactured.

### EMBODIMENT

Here will be described on an embodiment according to the present invention referring to comparative examples for comparison.

### (Embodiment)

In the embodiment, there is used an Nd-Fe-B-based magnet and alloy composition thereof is Nd/ Fe/ B= 32.7/ 65.96/ 1.34 in wt%. Polyisobutylene as binder and toluene as solvent have been used to prepare a binder solvent. The binder has been added to 100 grams of magnet powder so as to obtain slurry containing 16.7 wt% of binder with reference to the total weight of the magnet powder and the binder. After that, a green sheet having 4 mm thickness (as designed value) has been manufactured from thus obtained slurry by a slot-die system and the thus obtained green sheet has been die-cut into a desired shape for product. After calcination process, the formed green sheet has been sintered by SPS method. Other processes are the same as the processes in [Method for Manufacturing Permanent Magnet] mentioned above.

### (Comparative Example)

The doctor blade system has been employed to form a green sheet. Other conditions are the same as the embodiment.

### (Comparison of Embodiment and Comparative Example)

Here are compared the green sheets formed in the embodiment and in the comparative example. The thickness precision of the green sheet of the embodiment is superior to precision margin of error of plus or minus 1 % with reference to the designed value (4 mm). Meanwhile, the thickness precision of the green sheet of the comparative example is inferior to precision margin of error of plus or minus 5 % with reference to the designed value (4 mm) . That is, the formation of green sheet using the slot-die system can improve the thickness precision of the green sheet compared with the doctor blade system. As a result, in the embodiment, each formed body can be appropriately sintered without any variations in the pressure value or sintering temperature owing to the uniform thickness of formed bodies, even if the sintering process is executed in a state where a plurality of formed bodies (for instance, ten formed bodies) are put in the sintering die and simultaneously sintered. Meanwhile, in the comparative example, if the sintering is executed in a state where a plurality of formed bodies (for instance, ten formed bodies) are put in the sintering die and simultaneously sintered, as the formed bodies does not have a uniform thickness, variations in proper pressure values or proper sintering temperatures occur in respective formed body, and appropriate sintering cannot be achieved.

As described in the above, according to the permanent magnet 1 and the method for manufacturing the permanent magnet 1 directed to the embodiment, magnet material is milled into magnet powder. Next, the magnet powder and a binder are mixed to obtain a mixture (slurry or a powdery mixture) including 1 to 40 wt% of the binder therein. Next, by high precision coating of a substrate with the mixture, a green sheet is obtained at thickness precision within a margin of error of plus or minus 5% with reference to a designed value. Thereafter, the green sheet is held for predetermined time at binder decomposition temperature in non-oxidizing atmosphere, whereby depolymerization reaction changes the binder into monomer and thus removes the binder. The green sheet with the binder removed therefrom undergoes pressure sintering such as SPS method so as to obtain a permanent magnet 1. Accordingly, even if a plurality of formed bodies die-cut from the green sheet are sintered simultaneously, the formed bodies can be sintered satisfactorily; the thickness of each formed body is made uniform, which avoids variations in proper pressure values or proper sintering temperatures. As a result, improvement in productivity can be achieved.

Further, in the step of obtaining the green sheet, the mixture is coated with the substrate by using a slot die and thickness of a sheet thus coated with the mixture is measured so as to perform feed back control of a gap between the slot die and the substrate based on a measured thickness . Therefore, the thickness precision of the green sheet can further be improved.

Further, the permanent magnet 1 is a pressure-sintered magnet. Since pressure sintering allows sintering of the permanent magnet 1 at lower sintering temperature, grain growth at sintering is suppressed and magnetic performance can be improved. Further, the thus sintered magnet uniformly contracts and deformations such as warpage and depressions do not occur there. Further, the sintered magnet having uniformly contracted gets pressed uniformly, which eliminates adjustment process to be conventionally performed after sintering and simplifies manufacturing process. Thereby, a permanent magnet can be manufactured with dimensional accuracy. Further, even if above such permanent magnets are made thin in the course of manufacturing, increase in the number of manufacturing processes can be avoided without lowering a material yield.

Further, in the step of pressure sintering the green sheet, the green sheet is sintered by uniaxial pressure sintering such as SPS method. Therefore, the thus sintered magnet uniformly contracts and deformations such as warpage and depressions can be prevented in the magnet.

Further, in the step of pressure sintering the green sheet, the green sheet is sintered by electric current sintering such as SPS method. Thereby, quick heating and cooling can be realized and sintering in a lower temperature range can be realized, as well. As a result, the heating-up and holding periods in the sintering process can be shortened; so that a densely sintered body can be manufactured in which grain growth of the magnet particle is suppressed.

Further, before the step of pressure sintering the green sheet, the binder is decomposed and removed from the green sheet by holding the green sheet for a predetermined length of time at binder decomposition temperature in a non-oxidizing atmosphere. Thereby, carbon content in the magnet can be reduced previously. Consequently, previous reduction of carbon content can prevent alpha iron from separating out in a main phase of the sintered magnet and the entirety of the magnet can be sintered densely. Thereby, decrease in the coercive force can be prevented.

Further, in the step of calcinations, the green sheet to which the binder has been mixed is held in a hydrogen atmosphere or a mixed gas atmosphere of hydrogen and inert gas for a predetermined length of time at temperature range of 200 through 900 degrees Celsius, more preferably, at 400 through 600 degrees Celsius. Thereby, carbon content in the magnet can be reduced reliably.

Further, of magnet powder, milling condition, mixing condition, calcination condition, sintering condition. are not restricted to conditions described in the embodiment. For instance, in the above described embodiment, magnet material is dry-milled by using a jet mill. Alternatively, magnet material may be wet-milled by using a bead mill. In the above-mentioned embodiment, the green sheet is formed in accordance with a slot-die system. However, a green sheet may be formed in accordance with other system or molding (e.g., calendar roll system, comma coating system, extruding system, injection molding, doctor blade system.), as long as it is the system that is capable of forming slurry or fluid-state mixture into a green sheet on a substrate at high accuracy. Further, in the above embodiment, the magnet is sintered by SPS method, however, the magnet may be sintered by other pressure sintering methods (for instance, hot press sintering.).

Further, the calcination process may be omitted. Even so, the binder is thermally decomposed during the sintering process and certain extent of decarbonization effect can be expected. Alternatively, the calcination process may be performed in an atmosphere other than hydrogen atmosphere.

Although resin, long-chain hydrocarbon, fatty acid methyl ester are mentioned as examples of binders in the embodiment, other material may be used.

Description of the present invention has been given by taking the example of the Nd-Fe-B-based magnet. However, magnet made of other kinds of material (for instance, cobalt magnet, alnico magnet, ferrite magnet.) may be used. Further, in the embodiments of present invention, the proportion of Nd component ratio with reference to the alloy composition of the magnet is set higher in comparison with Nd component ratio in accordance with the stoichiometric composition. The proportion of Nd component may be set the same as the alloy composition according to the stoichiometric composition.

### DESCRIPTION OF REFERENCE NUMERALS AND SIGNS

- 1: permanent magnet
- 11: jet mill
- 12: slurry
- 13: green sheet
- 15: slot die
- 25: formed body
- 31: sintering die

## Claims

1. A manufacturing method of a Nd-Fe-B-based rare-earth permanent magnet comprising steps of:
milling magnet material into magnet powder;
preparing a mixture by mixing the magnet powder and a binder so that the binder is included at a rate of 1 to 40 wt% with reference to total weight of the magnet powder and the binder;
obtaining a green sheet by coating a surface of a substrate with the mixture by high precision coating so that a sheet-like-shaped green sheet has thickness precision within a margin of error of plus or minus 5% with reference to a designed value; and
pressure sintering the green sheet;
**characterized in that** in the step of obtaining the green sheet,
the substrate is coated with the mixture by using a slot die, and
thickness of the green sheet thus coated with the mixture is measured so as to perform feed back control of a gap between the slot die and the substrate based on a measured thickness.

2. The manufacturing method of a rare-earth permanent magnet according to claim 1, wherein, in the step of pressure sintering the green sheet, the green sheet is sintered by uniaxial pressure sintering.

3. The manufacturing method of a rare-earth permanent magnet according to claim 1, wherein, in the step of pressure sintering the green sheet, the green sheet is sintered by electric current sintering.

4. The manufacturing method of a rare-earth permanent magnet according to any of claims 1 through 3, wherein, before the step of pressure sintering the green sheet, the binder is decomposed and removed from the green sheet by holding the green sheet for a predetermined length of time at binder decomposition temperature in a non-oxidizing atmosphere.

5. The manufacturing method of a rare-earth permanent magnet according to claim 4, wherein, when decomposing and removing the binder from the green sheet, the green sheet is held for the predetermined length of time at temperature range of 200 degrees Celsius to 900 degrees Celsius in a hydrogen atmosphere or a mixed gas atmosphere of hydrogen and inert gas.

## Patentansprüche

1. Herstellungsverfahren für einen Nd-Fe-B-basierten Seltenerd-Permanentmagneten, das die folgenden Schritte umfasst:
Mahlen eines Magnetmaterials zu einem Magnetpulver,
Vorbereiten einer Mischung durch das Mischen des Magnetpulvers mit einem Bindemittel, sodass das Bindemittel mit einem Anteil von 1 bis 40 Gewichtsprozent in Bezug auf das Gesamtgewicht des Magnetpulvers und des Bindemittels enthalten ist,
Erhalten einer Grünschicht durch das Beschichten einer Fläche eines Substrats mit der Mischung durch eine Hochpräzisionsbeschichtung, sodass eine schichtartig geformte Grünschicht eine Dickenpräzision mit einer Fehlerspanne von ± 5% in Bezug auf einen vorgegebenen Wert aufweist, und
Drucksintern der Grünschicht,
**dadurch gekennzeichnet, dass** in dem Schritt zum Erhalten der Grünschicht:
das Substrat mit der Mischung unter Verwendung einer Schlitzdüse beschichtet wird, und
die Dicke der derart mit der Mischung beschichteten Grünschicht gemessen wird, um eine Regelung des Abstands zwischen der Schlitzdüse und dem Substrat basierend auf der gemessenen Dicke durchzuführen.

2. Herstellungsverfahren für einen Seltenerd-Permanentmagneten nach Anspruch 1, wobei in dem Schritt zum Drucksintern der Grünschicht die Grünschicht durch ein uniaxiales Drucksintern gesintert wird.

3. Herstellungsverfahren für einen Seltenerd-Permanentmagneten nach Anspruch 1, wobei in dem Schritt zum Drucksintern der Grünschicht die Grünschicht durch ein elektrisches Stromsintern gesintert wird.

4. Herstellungsverfahren für einen Seltenerd-Permanentmagneten nach einem der Ansprüche 1 bis 3, wobei, vor dem Schritt zum Drucksintern der Grünschicht das Bindemittel zersetzt und von der Grünschicht entfernt wird, indem die Grünschicht für eine vorbestimmte Zeitdauer bei einer Bindemittel-Zersetzungstemperatur in einer nicht-oxidierenden Atmosphäre gehalten wird.

5. Herstellungsverfahren für einen Seltenerd-Permanentmagneten nach Anspruch 4, wobei, wenn das Bindemittel zersetzt und von der Grünschicht entfernt wird, die Grünschicht für die vorbestimmte Zeitdauer in einem Temperaturbereich von 200 Grad Celsius bis 900 Grad Celsius in einer Wasserstoffatmosphäre oder einer Mischgasatmosphäre aus Wasserstoff und einem Inertgas gehalten wird.

## Revendications

1. Procédé de fabrication d'un aimant permanent à terres rares à base de Nd-Fe-B comprenant les étapes suivantes :
broyage d'un matériau d'aimant en une poudre d'aimant ;
préparation d'un mélange en mélangeant la poudre d'aimant avec un liant de telle sorte que le liant est inclus avec un pourcentage massique compris entre 1 % et 40 % par rapport à la masse totale de poudre d'aimant et de liant ;
obtention d'une feuille d'ébauche en enduisant une surface de substrat avec le mélange par enduction de haute précision de telle sorte que la marge d'erreur sur la précision de l'épaisseur de la feuille d'ébauche laminaire est de plus ou moins 5 % par rapport à une valeur de conception ; et
frittage sous pression de la feuille d'ébauche ;
**caractérisé en ce qu'**à l'étape d'obtention de la feuille d'ébauche,
le substrat est enduit du mélange en utilisant une filière plate, et
l'épaisseur de la feuille d'ébauche ainsi enduite avec le mélange est mesurée de manière à mettre en oeuvre un contrôle par rétroaction de l'intervalle entre la filière plate et le substrat sur base de l'épaisseur mesurée.

2. Procédé de fabrication d'un aimant permanent à terres rares selon la revendication 1, dans lequel, à l'étape de frittage sous pression de la feuille d'ébauche, la feuille d'ébauche est frittée par frittage sous pression uniaxiale.

3. Procédé de fabrication d'un aimant permanent à terres rares selon la revendication 1, dans lequel, à l'étape de frittage sous pression de la feuille d'ébauche, la feuille d'ébauche est frittée par frittage sous courant électrique.

4. Procédé de fabrication d'un aimant permanent à terres rares selon l'une quelconque des revendications 1 à 3, dans lequel, avant l'étape de frittage sous pression de la feuille d'ébauche, le liant est décomposé et éliminé de la feuille d'ébauche en maintenant la feuille d'ébauche durant une période prédéterminée à une température de décomposition du liant sous atmosphère non oxydante.

5. Procédé de fabrication d'un aimant permanent à terres rares selon la revendication 4, dans lequel, lors de la décomposition et de l'élimination du liant de la feuille d'ébauche, la feuille d'ébauche est maintenue durant une période prédéterminée dans une plage de température comprise entre 200 degrés Celsius et 900 degrés Celsius sous une atmosphère d'hydrogène ou sous une atmosphère de mélange gazeux d'hydrogène et de gaz inerte.
